# EUROPEAN PATENT SPECIFICATION

(11) **EP 0 946 778 B1**
(45) Date of publication and mention of the grant of the patent: **22.08.2001**
(21) Application number: 97911364.4
(22) Date of filing: 07.11.1997
(51) Int. Cl.: C23C 4/18, B22D 11/04

(54) **COATING OF CONTINUOUS CASTING MACHINE COMPONENTS**
VERFAHREN ZUM BESCHICHTEN VON BAUTEILEN EINER STRANGGIESSANLAGE
REVETEMENT DE COMPOSANTS DE MACHINE A MOULAGE CONTINU

(30) Priority: 08.11.1996 GB 9623344
(43) Date of publication of application: 06.10.1999
(73) Proprietor: Monitor Coatings and Engineers Limited (Cy.nr. 3306972), Wallsend, Tyne & Wear NE28 7RD (GB)
(72) Inventor: LAVIN, Philip, Anthony, Northumberland NE46 2HN (GB)
(74) Representative: Godwin, Edgar James
(86) International application number: GB9703073
(87) International publication number: WO9821379

(56) References cited:
- EP-A- 0 383 934
- EP-A- 0 569 585
- FR-A- 2 388 618
- GB-A- 2 269 392
- PATENT ABSTRACTS OF JAPAN vol. 010, no. 081 (M-465), 29 March 1986 & JP 60 221151 A (KAWASAKI SEITETSU KK), 5 November 1985,
- PATENT ABSTRACTS OF JAPAN vol. 014, no. 262 (M-0981), 6 June 1990 & JP 02 075447 A (NOMURA TECHNO RES KK), 15 March 1990,

## Description

This invention relates to the coating of components used in the continuous casting of ferrous and non-ferrous materials.

The topmost stage of a continuous casting machine is composed of a hollow box made up of side plates and end plates (and sometimes a central divider), usually of copper, which are water cooled, At the initial stage of casting a plug or dummy bar is positioned at the bottom of the mould and molten metal is poured into the mould from a ladle via a tundish. The water-cooled copper walls of the mould and the cold surface of the plug create a thin solidified skin which contains the molten material. As the molten metal continuous to solidify, the plug is slowly withdrawn downwards from the mould zone whilst the level of molten material at the top of the mould is maintained by continuously adding further molten material. A mould powder may be added simultaneously, to form a layer on the surface of the molten metal.

As the plug or dummy bar and the solidifying slab or strand to which it is now attached leaves the mould zone, it then enters a grid plate zone. The grid plates are usually made of cast iron or steel. Each grid plate comprises several raised "fingers" with surfaces which are in contact with the chilled skin of the slab and which continue to constrain the solidifying slab to the requisite cross-sectional shape whilst cooling water is continuously sprayed onto the surface of the slab in between the fingers. During the time of this transfer of the slab from the mould and through the grid plate zone, the thickness of the chilled skin is increasing.

The slab then passes further on down through the machine through a series of guides and rolls, which continue to constrain the slab to the designed shape. Whilst passing down the casting machine the plane of the slab is gradually changed from a vertical direction to a horizontal direction until the fully solidified but still hot slab emerges on a conveyor table at the bottom of the machine, where it is cut to the requisite length.

The surfaces of both the mould components and the grid plates are subject to severe wear due to the abrasive, adhesive, and erosive wear mechanisms induced by the high ferrostatic pressures, the high temperatures, and the formation of oxide skins and exacerbated by the entrainment of extraneous third body particles. In a relatively short time, these components become so worn that they are unable to constrain the slab to the correct size and shape. The casting campaign then has to be terminated whilst new or refurbished parts are fitted. Thus the severe wear of these critical components limits the casting time and therefore the efficiency of the continuous casting process.

GB-A-2 269 392 discloses a method of protecting a metallic component against wear by applying to the component, by flame spraying, a coating consisting of ceramo-metallic material. The coating is treated by the technique described in GB-A-1 466 074 (see below).

JP-A-60 221 151 discloses a continuous casting mould having a thermal spray coating of ceramo-metallic material. The surface is preliminarily subjected to Ni plating or a surface treatment in which Ni-W-Fe alloy is plated on the Ni plating over at least a half region from the lowe part.

JP-A-02 075 447 discloses a continuous casting mould with a thermal spray coating of ceramo-metallic material.

There is a need for a method of coating capable of withstanding the aggressive high temperature wear environment, thus extending the length of the normal continuous casting campaign.

In one aspect the present invention provides a method of protecting a wall component for a continuous casting mould against wear, the method comprising applying to an internal surface of the mould wall component, by flame spraying, a coating consisting of ceramo-metallic material, the coating having a thickness which increases progressively from a first region of the internal surface adjacent one end of the mould wall component, which is the upper end when in use, to a second region adjacent the opposite end, which is the lower end when in use.

The internal surface of the mould wall component is the surface which confines the metal being cast.

The method comprises the following steps: a) applying to an internal surface of the mould wall component, by flame spraying, a rough first coating consisting of ceramo-metallic material, the first coating having a thickness which increases progressively from a first region of the internal surface adjacent one end of the mould wall component, which is the upper end when in use, to a second region adjacent the opposite end, which is the lower end when in use; b) applying a ceramic slurry to the first coating; c) heating the ceramic slurry to form a second coating consisting of ceramic material; d) removing excess ceramic material from the second coating to produce a composite ceramo-metallic and ceramic surface; e) impregnating the composite surface with a solution of at least one soluble compound capable of being converted, on heating, into an insoluble substance which bonds the coatings, the soluble compound being selected from chromia and phosphate forming compounds capable of being converted into oxides and phosphates on heating; and f) heating the coatings to cause bonding and densification of the coatings by the said substance; whereby a composite coating is produced having a thickness which increases progressively from the said first region to the said second region of the internal surface of the mould wall component.

In another aspect, the present invention provides a method of protecting a grid plate for a continuous casting machine against wear, the method comprising applying to a strand-confining surface of the grid plate, by flame spraying, a coating consisting of ceramo-metallic material, the coating being in the form of an array of mutually isolated islands of the ceramo-metallic material.

The method in this aspect comprises the following steps: a) applying to a strand-confining surface of the grid plate, by flame spraying, a rough first coating consisting of ceramo-metallic material, the first coating being in the form of an array of mutually isolated islands of the ceramo-metallic material; b) applying a ceramic slurry to the islands of ceramo-metallic material; c) heating the ceramic slurry to form a second coating consisting of ceramic material; d) removing excess ceramic material from the second coating to produce a composite ceramo-metallic and ceramic surface; e) impregnating the composite surface with a solution of at least one soluble compound capable of being converted, on heating, into an insoluble substance which bonds the coatings, the soluble compound being selected from chromia and phosphate forming compounds capable of being converted into oxides and phosphates on heating; and f) heating the coatings to cause bonding and densification of the coatings by the said substance; whereby a composite coating is produced which is in the form of an array of mutually isolated islands.

The final ceramic coating of both methods is preferably a so-called Monitox coating, which is achieved by applying to a substrate a slurry containing a chromium compound capable of being converted into a chromium oxide and/or a chromium phosphate at temperatures of at least 250°C, heating the slurry (e.g. at about 260°C) to produce a porous ceramic coating, and then densifying and bonding the coating by one or more process cycles comprising impregnating the porous coating with at least one chromia or phosphate forming solution, removing excess impregnant, and heating. Such a technique is described in GB-A-1 466 074, for example.

The first coating may be any cermet (ceramo-metallic) coating but is preferably a tungsten carbide cobalt coating and is preferably applied in several successive layers. The flame spraying process is preferably a high velocity oxygen-liquid fuel process which is often referred to as an HVOF process. This process is a commercially available flame spraying process in which fuel and oxygen are combusted in a specially designed chamber which is connected to a water-cooled tube or nozzle at the combustion chamber exit. The combustion products are accelerated down the nozzle, constituting a gun or torch. Powdered materials of closely controlled sizes are metered into the gun and are thus accelerated and heated as they pass along the hot high-velocity gas stream. Upon impacting with the substrate at a specific distance from the gun the particles splat and build up upon each other and the substrate to form a highly bonded and dense coating. Various coatings can be produced in this manner but a tungsten carbide 17% cobalt coating is the preferred coating for applying to the casting machine components.

All flame sprayed coatings to a greater or lesser degree contain micro-cracks or fissures which are the result of the quench stresses generated as the hot high velocity particles impact upon the substrate Sometimes these micro-cracks can be extremely small, to such an extent that they are very difficult to discern using normal metallographic techniques. However, these very small cracks can propagate under the superimposed thermally and mechanically generated stresses and unless they can be effectively 'locked' or 'keyed' the coating will eventually fail by progressive spallation. The Monitox coating process induces the growth of oxides within these very small fissures and thus creates a resistance to crack propagation.

The Monitox coating is applied in an aqueous slurry form containing various oxides and chemicals. This layer is then dried and heated (250 to 500°C). At this stage is 'soft' in that it is a collection of hard particles which are not very well bonded to each other or to the substrate. Thus, at this stage, excess coating can easily be removed by scraping or sanding operations so as to reveal the peaks of the underlying tungsten carbide coating which, in the 'as sprayed' condition, exhibits a coarse surface somewhat like a coarse sandpaper. Thus, a relatively smooth composite surface can be produced which comprises areas of ceramic and carbide material. This composite surface is then further densified and hardened by a cyclic process of impregnation and further heat treatment; for example from 3 to 10 cycles of impregnation and heat treatment can be required.

When applying the composite coating to the mould components it has been found to be surprisingly beneficial to deposit the first coating to a tapered thickness profile from the top of each component to the bottom. The hottest region of the end and side plates is at the top at the meniscus zone. The inventor believes that making the coating thin in this area accommodates and withstands the high thermal stresses imposed in this area. The inventor also believes that making the coating thicker towards the lower end of the walls resists ferrostatic pressures and prevents the underlying ductile material from deforming under the applied load; if the coating is too thin in this area, deformation of the material allows the now unsupported and brittle tungsten carbide material to crack, and then these cracks can be propagated along any layers of weakness within the coating or along the coating/substrate interface, eventually causing the coating to spall from the copper surface. A suitable variable coating thickness profile has been found to be a substantially linear increase from 0.08 mm (0.003 inch) at the top to 0.46 mm (0.018 inch) at the bottom, although other thickness variations may be preferred depending upon the temperature and pressure characteristics of the casting process.

It is preferable for the coating to extend over the whole height of each mould component. However, the coating may terminate below the upper edge of the mould wall, provided it extends above the highest level of the molten metal. The coating may have a substantially constant thickness in an upper region adjacent the upper edge of the mould wall component; it may have a substantially constant thickness in a lower region adherent the lower edge of the mould wall component; and the thickness may increase progressively in a linear manner, an exponential manner, or any other suitable manner between the upper and lower regions. The minimum thickness is chosen primarily having regard to heat transfer, preferably in the range from 0.05 to 0.1 mm. The maximum thickness is chosen having regard to mechanical strength as well as heat transfer, preferably in the range from 0.4 to 1.0 mm.

When coating the grid plates, it has been found to be surprisingly beneficial to form a pattern of separate islands. It appears that any particular thickness may be applied, but a thickness of approx. 0.38 mm (0.015 inch) is presently preferred. It has been found to be particularly beneficial to deposit the coating in an island pattern in which each island is approx. 5 mm square or 5 mm in diameter; each island is defined at its perimeter by an uncoated band approx. 2 mm wide. The inventor believes that the island pattern allows the coating to accommodate the high thermal stresses which are imposed on the grid plates during service, thus preventing premature coating failure by spallation. A suitable thickness range may be from 0.3 to 0.5 mm. The transverse dimensions of the islands may conveniently be in the range from 4 to 8 mm, the islands being spaced apart by 1 to 3 mm, for example.

The invention will be described further, by way of example with reference to the accompanying drawing, whose sole Figure schematically shows the internal surface of a grid plate.

### Example 1: Process for coating grid plates

(1) Degrease the grid plates.
(2) Mask where no coating is required.
(3) Grit-blast.
(4) Apply WC - 17% Co coating to the fingers of the grid plates by HVOF using masking devices to ensure the requisite 'island pattern'.
(5) Re-mask.
(6) Apply Monitox slurry.
(7) Fire at approx. 250 to 300°C.
(8) Cool.
(9) Remove excess ceramic.
(10) Impregnate the coatings with oxide or phosphate forming compounds.
(11) Fire at approx. 250 to 300°C.
(12) Repeat operations (10) and (11) for 3 to 10 cycles.

The drawing shows a cast iron grid plate 1 with gaps 2, through which cooling water is sprayed, and raised fingers 3 provided with the composite coating 4 made up of a pattern of rectangular islands 5 (approx. 5 mm square, separated by at least 1 mm).

### Example 2: Process for coating copper mould components

(1) Degrease the components.
(2) Mask where no coating is required.
(3) Grit-blast.
(4) Apply WC - 17% Co coating using computer-controlled robotic manipulation so as to ensure that the required tapered thickness profile (linearly increasing from 0.08 mm to 0.46 mm) is obtained from top to bottom on each component.
(5) Re-mask.
(6) Apply Monitox slurry.
(7) Fire at approx. 250 to 300°C.
(8) Cool.
(9) Remove excess ceramic.
(10) Impregnate the coatings with oxide or phosphate forming compounds.
(11) Fire at approx. 250 to 300°C,
(12) Repeat operations (10) and (11) for 3 to 10 cycles.

## Claims

1. A method of protecting a wall component for a continuous casting mould against wear, the method comprising:
a) applying to an internal surface of the mould wall component, by flame spraying, a rough first coating consisting of ceramo-metallic material, the first coating having a thickness which increases progressively from a first region of the internal surface adjacent one end of the mould wall component, which is the upper end when in use, to a second region adjacent the opposite end, which is the lower end when in use.
b) applying a ceramic slurry to the first coating;
c) heating the ceramic slurry to form a second coating consisting of ceramic material;
d) removing excess ceramic material from the second coating to produce a composite ceramo-metallic and ceramic surface;
e) impregnating the composite surface with a solution of at least one soluble compound capable of being converted, on heating, into an insoluble substance which bonds the coatings, the soluble compound being selected from chromia and phosphate forming compounds capable of being converted into oxides and phosphates on heating; and
f) heating the coatings to cause bonding and densification of the coatings by the said substance;
whereby a composite coating is produced having a thickness which increases progressively from the said first region to the said second region of the internal surface of the mould wall component.

2. A method as claimed in claim 1, wherein the minimum thickness of the coating or the composite coating is 0.05 - 0.1 mm and the maximum thickness of the coating or the composite coating is 0.4 - 1.0 mm.

3. A method as claimed in claim 1 or 2, wherein the wall component is a copper end plate or side plate for a continuous casting mould.

4. A method of protecting a grid plate for a continuous casting machine against wear, the method comprising:
a) applying to a strand-confining surface of the grid plate, by flame spraying, a rough first coating consisting of ceramo-metallic material, the first coating being in the form of an array of mutually isolated islands of the ceramo-metallic material;
b) applying a ceramic slurry to the islands of ceramo-metallic material;
c) heating the ceramic slurry to form a second coating consisting of ceramic material;
d) removing excess ceramic material from the second coating to produce a composite ceramo-metallic and ceramic surface;
e) impregnating the composite surface with a solution of at least one soluble compound capable of being converted, on heating, into an insoluble substance which bonds the coatings, the soluble compound being selected from chromia and phosphate forming compounds capable of being converted into oxides and phosphates on heating; and
f) heating the coatings to cause bonding and densification of the coatings by the said substance;
whereby a composite coating is produced which is in the form of an array of mutually isolated islands.

5. A method as claimed in claim 4, wherein the islands are substantially square, preferably have a thickness of 0.3 - 0.5 mm, preferably have transverse dimensions in the range 4 - 8 mm, and are preferably spaced apart by 1 - 3 mm.

6. A method as claimed in any preceding claim, wherein the ceramic slurry contains a chromium compound capable of being converted into chromium oxide at a temperature of at least 250°C.

7. A method as claimed in any preceding claim, wherein the impregnation/heat treatment cycle of steps (e) and (f) is repeated.

8. A method as claimed in any preceding claim, wherein the ceramo-metallic material is applied by a high-velocity oxygen-liquid fuel process.

9. A method as claimed in any preceding claim, wherein the ceramo-metallic material contains a carbide, preferably tungsten carbide.

10. A method as claimed in claim 9, wherein the ceramo-metallic material contains cobalt.

## Patentansprüche

1. Verfahren zum Schützen einer Wandkomponente für eine kontinuierliche Gießform gegen Abnutzung, wobei das Verfahren umfaßt
a) Aufbringen auf eine Innenoberfläche der Formwandkomponente durch Flammsprühen einen ersten Rohüberzug, der aus keramisch-metallischem Material . besteht, wobei der erste Überzug eine Dicke hat, die sich fortschreitend von einem ersten Bereich der Innenoberfläche benachbart zu einem Ende der Formwandkomponente, welches das obere Ende, wenn in Benutzung, ist, zu einem zweiten Bereich, benachbart zu dem entgegengesetzten Ende, welches das untere Ende, wenn in Benutzung, ist, erhöht,
b) Aufbringen einer Keramikaufschlämmung auf den ersten Überzug,
c) Erhitzen der Keramikaufschlämmung unter Bilden eines zweiten Überzugs, der aus Keramikmaterial besteht,
d) Entfernen von Überschuß Keramikmaterial von dem zweiten Überzug unter Herstellen einer keramisch-metallischen und keramischen Verbundoberfläche,
e) Imprägnieren der Verbundoberfläche mit einer Lösung mindestens einer löslichen Verbindung, die fähig ist, bei Erhitzen in eine unlösliche Substanz umgewandelt zu werden, die die Überzüge bindet, wobei die lösliche Verbindung ausgewählt ist aus Chromoxid und Phosphat bildenden Verbindungen, fähig, in Oxide und Phosphate bei Erhitzen umgewandelt zu werden, und
f) Erhitzen der Überzüge unter Erzeugen von Binden und Verdichtung der Überzüge durch die Substanz,
wodurch ein Verbundüberzug mit einer Dicke hergestellt wird, die sich fortschreitend von dem ersten Bereich zu dem zweiten Bereich der Innenoberfläche der Formwandkomponente erhöht.

2. Verfahren nach Anspruch 1, wobei die Minimumdicke des Überzugs oder des Verbundüberzugs 0,05 - 0,1 mm beträgt, und die maximale Dicke des Überzugs oder des Verbundüberzugs beträgt 0,4 - 1,0 mm.

3. Verfahren nach Anspruch 1 oder 2, wobei die Wandkomponente eine Kupferendplatte oder Seitenplatte für eine kontinuierliche Gießform ist.

4. Verfahren zum Schützen einer Gitterplatte für eine kontinuierliche Gießmaschine gegen Abnutzung, wobei das Verfahren umfaßt
a) Aufbringen auf eine Strangabsperroberfläche der Gitterplatte durch Flammsprühen einen ersten Rohüberzug, aus keramisch-metallischem Material bestehend, wobei der erste Überzug in der Form einer Reihe von gegenseitig isolierten Inseln des keramisch-metallischen Materials ist,
b) Aufbringen einer keramischen Aufschlämmung auf die Inseln von keramisch-metallischem Material,
c) Erhitzen der keramischen Aufschlämmung unter Bilden eines zweiten Überzugs, der aus Keramikmaterial besteht,
d) Entfernen von Überschuß von Keramikmaterial von dem zweiten Überzug unter Herstellen einer keramisch-metallischen und keramischen Verbundoberfläche,
e) Imprägnieren der Verbundoberfläche mit einer Lösung mindestens einer löslichen Verbindung, fähig, bei Erhitzen in eine unlösliche Substanz umgewandelt zu werden, die die Überzüge bindet, wobei die lösliche Verbindung ausgewählt ist aus Chromoxid und Phosphat bildenden Verbindungen, fähig, in Oxide und Phosphate bei Erhitzen umgewandelt zu werden, und
f) Erhitzen der Überzüge unter Erzeugen von Binden und Verdichtung der Überzüge durch die Substanz,
wodurch ein Verbundüberzug hergestellt wird, der in der Form einer Reihe von gegenseitig isolierten Inseln ist.

5. Verfahren nach Anspruch 4, wobei die Inseln im wesentlichen rechteckig sind, vorzugsweise eine Dicke von 0,3 - 0,5 mm haben, vorzugsweise querlaufende Dimensionen im Bereich von 4 - 8 mm haben, und vorzugsweise mit Abstand von 1 - 3 mm angeordnet sind.

6. Verfahren nach einem vorhergehenden Anspruch, wobei die keramische Aufschlämmung eine Chromverbindung enthält, fähig, in Chromoxid bei einer Temperatur von mindestens 250°C umgewandelt zu werden.

7. Verfahren nach einem vorhergehenden Anspruch, wobei der Imprägnierungs/Hitzebehandlungszyklus von Stufen (e) und (f) wiederholt wird.

8. Verfahren nach einem vorhergehenden Anspruch, wobei das keramisch-metallische Material durch ein Hochgeschwindigkeits-Sauerstoff-Flüssigkeit-Brennstoffverfahren aufgebracht wird.

9. Verfahren nach einem vorhergehenden Anspruch, wobei das kermisch-metallische Material ein Carbid, vorzugsweise Wolframcarbid, enthält.

10. Verfahren nach Anspruch 9, wobei das keramisch-metallische Material Kobalt enthält.

## Revendications

1. Procédé pour la protection d'un composant de paroi destiné à un moule de coulée continue contre l'usure, le procédé comprenant:
a) l'application sur une surface interne du composant de paroi du moule, par projection à chaud, d'un premier revêtement rugueux constitué d'un matériau céramo-métallique, le premier revêtement possédant une épaisseur qui augmente progressivement à partir d'une première zone de la surface interne adjacente à une extrémité du composant de paroi du moule, qui est l'extrémité supérieure pendant l'usage, vers une deuxième zone adjacente à l'extrémité opposée, qui est l'extrémité inférieure pendant l'usage;
b) l'application d'une suspension céramique épaisse sur le premier revêtement;
c) le chauffage de la suspension céramique épaisse pour former un deuxième revêtement constitué d'un matériau céramique;
d) le retrait de l'excès de matériau céramique provenant du deuxième revêtement pour produire une surface composite céramo-métallique et céramique;
e) l'imprégnation de la surface composite avec une solution d'au moins un composé soluble capable d'être converti, à la suite d'un chauffage, en une substance insoluble qui lie les revêtements, le composé soluble étant choisi parmi des composés formant un oxyde de chrome et un phosphate capables d'être convertis en oxydes et en phosphates à la suite d'un chauffage; et
f) le chauffage des revêtements pour entraîner la liaison et la densification des revêtements par ladite substance;
en conséquence de quoi, un revêtement composite est produit possédant une épaisseur qui augmente progressivement à partir de ladite première zone vers ladite deuxième zone de la surface interne du composant de paroi du moule.

2. Procédé suivant la revendication 1, dans lequel l'épaisseur minimum du revêtement ou du revêtement composite est de 0,05-0,1 mm et l'épaisseur maximum du revêtement ou du revêtement composite est de 0,4-1,0 mm.

3. Procédé suivant la revendication 1 ou 2, dans lequel le composant de paroi est une plaque d'extrémité ou une plaque latérale en cuivre destinée à un moule de coulée continue.

4. Procédé pour la protection d'une plaque-grille destinée à une machine de coulée continue contre l'usure, le procédé comprenant:
a) l'application sur une surface limitant la ligne de coulée continue de la plaque-grille, par projection à chaud, d'un premier revêtement rugueux constitué d'un matériau céramo-métallique, le premier revêtement étant sous la forme d'un ensemble d'îlots isolés mutuellement de matériau céramo-métallique;
b) l'application d'une suspension céramique épaisse sur les îlots de matériau céramo-métallique;
c) le chauffage de la suspension céramique épaisse pour former un deuxième revêtement constitué de matériau céramique;
d) le retrait de l'excès de matériau céramique provenant du deuxième revêtement pour produire une surface composite céramo-métallique et céramique;
e) l'imprégnation de la surface composite avec une solution d'au moins un composé soluble capable d'être converti, à la suite d'un chauffage, en une substance insoluble qui lie les revêtements, le composé soluble étant choisi parmi des composés formant un oxyde de chrome et un phosphate capables d'être convertis en oxydes et en phosphates à la suite d'un chauffage; et
f) le chauffage des revêtements pour entraîner la liaison et la densification des revêtements par ladite substance;
en conséquence de quoi, un revêtement composite est produit qui se trouve sous la forme d'un ensemble d'îlots isolés mutuellement.

5. Procédé suivant la revendication 4, dans lequel les îlots sont substantiellement carrés, possèdent de préférence une épaisseur de 0,3-0,5 mm, présentent de préférence des dimensions transversales dans l'intervalle de 4-8 mm et sont de préférence espacés par intervalle de 1-3 mm.

6. Procédé suivant l'une quelconque des revendications précédentes, dans lequel la suspension céramique épaisse contient un composé du chrome capable d'être converti en oxyde de chrome à une température d'au moins 250°C.

7. Procédé suivant l'une quelconque des revendications précédentes, dans lequel le cycle de traitement d'imprégnation/chauffage des étapes (e) et (f) est répété.

8. Procédé suivant l'une quelconque des revendications précédentes, dans lequel le matériau céramo-métallique est appliqué par un procédé à combustible liquide-oxygène à vitesse élevée.

9. Procédé suivant l'une quelconque des revendications précédentes, dans lequel le matériau céramo-métallique contient un carbure, de préférence un carbure de tungstène.

10. Procédé suivant la revendication 9, dans lequel le matériau céramo-métallique contient du cobalt.
